# EUROPEAN PATENT SPECIFICATION

(11) **EP 0 847 455 B1**
(45) Date of publication and mention of the grant of the patent: **06.05.1999**
(21) Application number: 96928616.0
(22) Date of filing: 30.08.1996
(51) Int. Cl.: C25D 15/00, B24D 18/00

(54) **PRODUCTION OF DIAMOND DRESSERS**
HERSTELLUNG VON SCHLEIFWERKZEUGEN
FABRICATION DE DRESSEURS AU DIAMANT

(30) Priority: 01.09.1995 GB 9517854
(43) Date of publication of application: 17.06.1998
(73) Proprietor: Consort Precision Diamond Company Limited, Kimmel Bay, Rhyl, Clwyd LL18 5JA (GB)
(72) Inventor: MORRIS, Peter, David, Abergele Clwyd LL22 7AT (GB); NOAKES, Stephen, Leslie, Colwyn Bay Clwyd LL29 7ES (GB)
(74) Representative: Lyons, Andrew John
(86) International application number: GB9602132
(87) International publication number: WO9709469

(56) References cited:
- US-A- 4 737 162

## Description

This invention concerns the production of diamond dressers.

Diamond dressers, sometimes known as diamond profile rolls, are mainly used in the aero engine and motor engine manufacturing industries. A diamond dresser is generally circular in shape with its periphery coated with diamonds to a predetermined configuration of high tolerance. A diamond dresser is mounted on a grinding machine and rotated by means of an independent drive unit to dress the configuration of the dresser onto a rotating abrasive (grinding) wheel. The grinding wheel is then ready for use in forming and finishing components especially of aero- and motor engines.

Diamond dressers are generally made by first forming a graphite mould to high accuracy, the internal profile of the mould matching the desired external profile of the finished diamond dresser. Diamonds are then adhered onto the internal surface of the mould and the mould is placed in a bath of electrolyte. The mould forms the cathode and a basket of nickel pellets form the anode, so that nickel is deposited on the diamond layer by an electro-plating process. The electro-plating process is continued until a layer of nickel of sufficient depth has been deposited on the diamonds. A solid steel shaft is then fitted in the centre of the mould using a low melting alloy. When the mould has cooled, the end faces of the mould are machined in a lathe and the graphite mould broken away to leave the diamond dresser.

US Patent Specification No. 4737162 discloses a method of producing precision abrasive articles by electroforming for use in metal removal operations. In this method diamond particles are packed firm between the inner circumferential surface of a mould and a centrally located metallic grid. Electrolyte for metal deposition, selected from Ni, Cu, Fe, Sn and Ag, is then pumped from a reservoir into the space containing the abrasive diamond particles. An electrical cathode connection is made to the mould and an anodic connection made to the anode. Metallic deposition around the diamond particles occurs on the inner annular surface of the mould and continues until a matrix supporting the diamond particles is formed. The mould with the matrix is then removed to receive the core material and the core is then machined to finished dimensions. The method is carried out at temperatures up to 93.3°C and without any movement of the mould.

To avoid a build up of stress or porosity in the nickel and to avoid excessive over plating, the electro-plating process is carried out slowly at a low current density. Typically the electro-plating process can take as long as 32 days. That length of time increases costs and causes considerable delays between receipt of and completion of an order for a diamond dresser. Furthermore, each electro-plating process requires a large area of operation as each mould has to be in its own electrolyte bath and each bath requires a heating jacket to bring the electrolyte up to a suitable operating temperature.

An object of this invention is to provide an improved process and apparatus for producing diamond dressers.

According to a first aspect of this invention, there is provided a process for producing diamond dressers including the steps of forming a mould for the dresser having a desired internal profile, adhering diamonds to said profile, and electro-plating a metal, typically nickel, onto the diamonds, characterised in that the electro-plating process is carried out while a swirling motion is imparted to the electrolyte.

According to a second aspect of this invention there is provided apparatus for producing diamond dressers comprising an electrolyte bath for receiving a mould of graphite having a desired internal profile coated with diamonds as cathode, a metal source, typically nickel, as anode and means for passing current between the anode and cathode, whereby metal is deposited on the diamonds, characterised by means for imparting a swirling motion to the electrolyte.

A swirling motion may be imparted to the electrolyte in any suitable way and preferably comprises pumping means. The electrolyte is preferably pumped through a plate having angled passages for the electrolyte. These passages preferably have an entrance on one radius and an exit on another radius spaced axially from the one radius in order to impart the swirling motion to the electrolyte.

It is believed that agitation of the electrolyte by imparting a swirling motion thereto in the mould eliminates air entrapment in the metal coating and hence reduces porosity. Furthermore, nodule formations on the metal coating may be reduced or ever eliminated because of the agitation. Further, it has been found that the invention can produce required nickel depths on the diamonds within a much shorter time period than hitherto. Typically a desirable depth of nickel may be achieved in under 7 days and even in about 3¹/₂ days.

The electrolyte bath is preferably maintained at a temperature above 35°C. Lower temperatures tend to result in uneven nickel growth on the diamonds. The electrolyte temperature is preferably in the range of 39 to 41°C.

The electrolyte for nickel plating is preferably nickel sulfamate ideally at a concentration in the range of 550 to 650 g/litre. The electrolyte may contain hardener and other additives, typically boric acid, nickel chloride and wetting agent. The electrolyte preferably has an acidic pH of above 3.5.

The diamonds may be adhered to the graphite mould in any suitable way. A conductive adhesive is preferably used for this purpose, such as a silver based adhesive, especially a silver loaded epoxy adhesive.

The nickel used for the electro-plating process is preferably in the form of pellets. These are ideally contained in a basket in the electrolyte within the graphite mould. The basket is preferably made of a conductive material that is not reactive with nickel The preferred basket for use in the invention is made of titanium.

The electro-plating process is preferably commenced at low current, which may be dependent on the area to be plated. The larger the area to be plated, the higher is the current used. Typically the start current used will be in the region of 2 amps and will be raised incremently up to 12-14 amps. The start current may be maintained for 16-24 hours and the final current may be maintained for up to 48 hours.

This gradual raising of the current may be achieved manually ie with regular attendance at the apparatus to adjust manually the current up to the maximum current to be used. It is preferred, however, that such raising of the current be independently controlled, so that attendance at the apparatus can be kept to a minimum. Preferably the raising of the current is pulsed, in other words, a constant current is preferably switched from one level to another in a predetermined, especially regular, manner. Raising of the current is preferably controlled by a microprocessor or computer.

It is believed that pulsed electro-plating may have several advantages. These advantages include that the metal (nickel) deposited will be finer, purer and smoother. Secondly by raising the limiting current density, the rate of metal (nickel) deposition may be increased. Thirdly, there may be improved metal adhesion to the substrate. Fourthly, a better plating distribution may be achieved. Finally, with a programmable means for raising the current, the electro-plating process may be commenced at any time during the working day and left to reach its maximum operating current at any desired time day or night.

Once a desired depth of metal, such as nickel, has been deposited in the mould, the mould can be removed from the electrolyte bath and finished in the usual way.

Traditionally only a single diamond dresser mould is electro-processed at a time in an electrolyte bath. It has now been found that a multiple diamond dresser mould can be processed in a single bath using the present invention. After electro-processing the mould is split and each part finished conventionally.

This invention will now be further described, by way of example only, with reference to the accompanying drawings, in which:-
Figure 1 shows schematically a prior art apparatus for producing a diamond dresser;
Figure 2 shows schematically an apparatus according to the invention for producing a diamond dresser; and
Figure 3 is a section through apparatus of the invention for producing multiple diamond dressers in a single operation.

Referring to Figure 1 of the accompanying drawings, a diamond dresser is produced conventionally, in the following manner. A graphite mould 10 is prepared having an internal profile 12 matching the desired outer profile of the diamond dresser to be made. A coating 14 of diamonds is adhered to the profile 12 using a conductive adhesive. The diamond coated mould 10 is placed in a bath of electrolyte 16 comprising an aqueous solution of nickel sulfamate. Within the mould 10 is placed a porous ceramic tube 18 within which is placed a titanium basket 20 containing nickel pellets 22. The nickel pellets form the anode and the mould 10 the cathode of an electrolytic cell. A constant current is applied across the anode and cathode for a sufficient period of time to deposit by electro-plating a layer of nickel 25 on the diamonds of a desired thickness. Usually the deposition period will be around 30-35 days. Periodically, the titanium basket of nickel pellets is replaced by a bianode, so that the basket can be flushed with water to remove debris. Also, the pH of the electrolyte is checked daily. Attempts to reduce the electro-plating time by increasing current density have proved unsuccessful. The resultant nickel coating was uneven, modular and pitted. In mould recesses nickel plating was found to be thinner than elsewhere.

After completion of the nickel plating, the mould is removed from the electrolyte bath, a steel shaft fixed in the centre of the mould using a low melting alloy and the graphite mould broken away. Finishing of end faces of the dresser on a lathe completes the production process.

Referring now to Figure 2 of the accompanying drawings it has been found that agitation of the electrolyte allows the current density to be increased and hence the electro-plating time to be reduced. A main difference according to the invention over the prior art process, as illustrated in Figure 2 of the drawings, is that the electrolyte 18 is pumped through a baffle plate 24 having angled passages 26 therethrough which are arranged to promote a swirling motion or turbulent flow pattern for the electrolyte through the mould. Thus, the passages 26 have a lower entry on one radius and an upper exit on a different radius, the respective radu being axially spaced from each other.

The electro-plating conditions used in the apparatus of Figure 2 were as follows:
Electrolyte: Nickel sulfamate with additions of boric acid, nickel chloride and wetting agent.
Electrolyte temperature: 40 ± 1°C.
Electrolyte pH: acidic above 3.5.
Current Density: dependent on surface area to be plated and to be increased gradually during plating period up to, for example 14 amps.
Electro-plating time: 3.5 days.

It was found that using a combination of electrolyte turbulence, higher electrolyte temperature than hitherto and higher current density than hitherto, a relatively uniform nickel coating could be achieved which was generally free of pitting.

Figure 3 of the accompanying drawings shows how the principles of the apparatus of Figure 2 can be extended to enable more than one diamond dresser to be made at one time. A bath 50 of nickel sulfamate electrolyte (as in Figure 2) contains a cylindrical plastics chamber 52 having a base 54 and a top 56.

The base 54 includes an inlet pipe 58 connected to a filter pump (not shown) leading to an entry flange 60 which encloses a multi-entry manifold 62. Above the manifold. 62 is a turbulence plate 64 having angled passages 66 therethrough for delivering electrolyte pumped from the electrolyte bath. The passages 66 are angled outward and upwards as well as into and out of the paper respectively in order to impart a swirling or turbulent motion to the electrolyte as it emerges into the chamber 52. Also from the base of the chamber are return pipes 68 for the electrolyte.

Seated on the turbulence plate 64 is a graphite mould 70 which has three dresser forms 70A, B and C leaving a gap between each. The internal profile of the mould is coated with diamonds 71 in the area of each dresser form. The diamonds being adhered using a silver loaded epoxy adhesive.

A porous ceramic tube 72 enclosing a titanium basket 74 containing nickel pellets 76 is fitted in the chamber 52 through its top 56 centrally of the mould 70. The titanium basket and the graphite mould are connected to a d.c. current supply as anode and cathode respectively.

The operating conditions for the apparatus of Figure 3 were substantially the same as for the apparatus of Figure 2, i.e. with the electrolyte being continuously pumped through the chamber 52. After completion of the electro-plating, the mould 70 is removed and the three dresser forms separated and finished off conventionally.

## Claims

1. A process for producing diamond dressers including the steps of forming a mould for the dresser having a desired internal profile, adhering diamonds to said profile, placing the mould in electrolyte, and electro-plating a metal onto the diamonds, characterized in that the electro-plating process is carried out while a swirling motion is imparted to the electrolyte.

2. A process as claimed in claim 1, characterized in that the electrolyte is pumped through the mould.

3. A process as claimed in claim 1 or 2, characterized in that the electrolyte is pumped through a plate having angled passages for the electrolyte.

4. A process as claimed in claim 3, characterized in that the passages have an entrance on one radius and an exit on another radius spaced axially from the one radius.

5. A process as claimed in any one of claims 1 to 4, characterized in that the electrolyte is maintained at a temperature above 35°C.

6. A process as claimed in claim 5, characterized in that the electrolyte temperature is maintained in the range of 39 to 41°C.

7. A process as claimed in any one of claims 1 to 6, characterized in that the metal is nickel.

8. A process as claimed in claim 7, characterized in that the electrolyte is aqueous nickel sulfamate.

9. A process as claimed in claim 8, characterized in that the electrolyte concentration is in the range of 550 to 650 g/litre.

10. A process as claimed in claim 8 or 9, characterized in that the electrolyte has an acidic pH of above 3.5.

11. A process as claimed in any one of claims 1 to 10, characterized in that the diamonds are adhered to the profile by means of a conductive adhesive.

12. A process as claimed in claim 11, characterized in that the adhesive is a silver based adhesive.

13. A process as claimed in claim 12, characterized in that the adhesive is a silver loaded epoxy adhesive.

14. A process as claimed in any one of claims 7 to 13, characterized in that the nickel is in the form of pellets.

15. A process as claimed in any one of claims 1 to 14, characterized in that the electro-plating is commenced at low current and raised gradually.

16. A process as claimed in claim 15, characterized in that the electro-plating is commenced at a current in the region of 2 amps.

17. A process as claimed in claim 15 or 16, characterized in that the current is raised to 12 to 14 amps.

18. A process as claimed in claim 15, 16 or 17, characterized in that the start current is maintained for 16 to 24 hours.

19. A process as claimed in any one of claims 1 to 18, characterized in that the final current is maintained for up to 48 hours.

20. A process as claimed in any one of claims 15 to 19, characterized in that raising of the current is pulsed.

21. Apparatus for producing diamond dressers comprising an electrolyte bath for receiving a mould of graphite having a desired internal profile coated with diamonds as cathode, a metal source as anode and means for passing electric current between the anode and cathode whereby metal is deposited on the diamonds, characterized by means for imparting a swirling motion to the electrolyte.

22. Apparatus as claimed in claim 21, characterized in that the means arranged to impart a swirling motion to the electrolyte comprises pump means.

23. Apparatus as claimed in claim 22, characterized by a plate through which the electrolyte is pumped, the plate having angled passages therethrough.

24. Apparatus as claimed in claim 23, characterized in that the passages of the plate have an entrance on one radius and an exit on another radius spaced axially from the one radius.

25. Apparatus as claimed in any one of claims 21 to 24, characterized by means for heating the electrolyte.

26. Apparatus as claimed in any one of claims 21 to 25, characterized in that the metal is contained in a basket in the electrolyte within the graphite mould.

27. Apparatus as claimed in claim 26, characterized in that the basket is made of conductive material that is not reactive with nickel.

28. Apparatus as claimed in claim 26 or 27, characterized in that the basket is made of titanium.

29. Apparatus as claimed in any one of claims 21 to 28 further characterized by means for altering the applied current.

30. Apparatus as claimed in claim 29, characterized by means for altering the applied current in a pulsed manner.

## Patentansprüche

1. Verfahren zum Herstellen von Diamant-Abrichtwerkzeugen mit den Schritten, eine Form für das Abrichtwerkzeug zu formen, welche ein erwünschtes inneres Profil aufweist, Diamanten an dem Profil anzukleben, die Form in einem Elektrolyten anzuordnen und die Diamanten elektrisch mit einem Metall zu plattieren,
dadurch **gekennzeichnet,**
daß der Vorgang des elektrischen Plattierens ausgeführt wird, während in den Elektrolyten eine Wirbelbewegung eingebracht wird.

2. Verfahren nach Anspruch 1,
dadurch **gekennzeichnet,**
daß der Elektrolyt durch die Form gepumpt wird.

3. Verfahren nach einem der Ansprüche 1 oder 2,
dadurch **gekennzeichnet**,
daß der Elektrolyt durch eine Platte mit gewinkelten Durchgängen für den Elektrolyten gepumpt wird.

4. Verfahren nach Anspruch 3,
dadurch **gekennzeichnet,**
daß die Durchgänge einen Eingang mit einem ersten Radius aufweisen, wobei ein Ausgang mit einem anderen Radius mit axialem Abstand zu dem ersten Radius angeordnet ist.

5. Verfahren nach einem der Ansprüche 1 bis 4,
dadurch **gekennzeichnet,**
daß der Elektrolyt auf einer Temperatur oberhalb von 35°C gehalten wird.

6. Verfahren nach Anspruch 5,
dadurch **gekennzeichnet,**
daß die Elektrolyttemperatur in dem Bereich zwischen 39 und 41°C gehalten wird.

7. Verfahren nach einem der Ansprüche 1 bis 6,
dadurch **gekennzeichnet**,
daß das Metall Nickel ist.

8. Verfahren nach Anspruch 7,
dadurch **gekennzeichnet,**
daß der Elektrolyt wässriges Nickelsulfamat ist.

9. Verfahren nach Anspruch 8,
dadurch **gekennzeichnet,**
daß die Elektrolytkonzentration im Bereich von 550 bis 650 g/Liter liegt.

10. Verfahren nach Anspruch 8 oder 9,
dadurch **gekennzeichnet,**
daß der Elektrolyt einen sauren pH-Wert oberhalb von 3,5 aufweist.

11. Verfahren nach einem der Ansprüche 1 bis 10,
dadurch **gekennzeichnet,**
daß die Diamanten an dem Profil mittels eines leitenden Klebers angeklebt werden.

12. Verfahren nach Anspruch 11,
dadurch **gekennzeichnet,**
daß der Kleber ein auf Silber basierender Kleber ist.

13. Verfahren nach Anspruch 12,
dadurch **gekennzeichnet,**
daß der Kleber ein mit Silber beladener Epoxid-Kleber ist.

14. Verfahren nach einem der Ansprüche 7 bis 13,
dadurch **gekennzeichnet,**
daß das Nickel die Form von Pellets aufweist.

15. Verfahren nach einem der Ansprüche 1 bis 14,
dadurch **gekennzeichnet,**
daß das elektrische Plattieren bei niedrigem Strom begonnen wird und dieser graduell erhöht wird.

16. Verfahren nach Anspruch 15,
dadurch **gekennzeichnet,**
daß das elektrische Plattieren bei einem Strom im Bereich von 2 Ampere begonnen wird.

17. Verfahren nach Anspruch 15 oder 16,
dadurch **gekennzeichnet,**
daß der Strom auf 12 bis 14 Ampere erhöht wird.

18. Verfahren nach einem der Ansprüche 15, 16 oder 17,
dadurch **gekennzeichnet,**
daß der Anfangsstrom über 16 bis 24 Stunden aufrechterhalten wird.

19. Verfahren nach einem der Ansprüche 1 bis 18,
dadurch **gekennzeichnet,**
daß der Endstrom bis zu 48 Stunden aufrechterhalten wird.

20. Verfahren nach einem der Ansprüche 15 bis 19,
dadurch **gekennzeichnet**,
daß die Erhöhung des Stroms gepulst ist.

21. Vorrichtung zum Herstellen von Diamant-Abrichtwerkzeugen mit einem Elektrolytbad zum Aufnehmen einer Form aus Graphit, die ein erwünschtes inneres, mit Diamanten beschichtetes Profil als Kathode aufweist, einer Metallquelle als Anode und Mitteln zum Leiten eines elektrischen Stroms zwischen der Anode und der Kathode, wobei Metall auf den Diamanten abgeschieden wird,
**gekennzeichnet** durch
Mittel zum Einbringen einer wirbelbewegung in den Elektrolyten.

22. Vorrichtung nach Anspruch 21,
dadurch **gekennzeichnet,**
daß die Mittel, die zum Einbringen einer Wirbelbewegung in den Elektrolyten vorgesehen sind, Pumpenmittel aufweisen.

23. Vorrichtung nach Anspruch 22,
**gekennzeichnet** durch
eine Platte, durch welche der Elektrolyt gepumpt wird, wobei die Platte gewinkelte Durchgänge aufweist.

24. Vorrichtung nach Anspruch 23,
dadurch **gekennzeichnet,**
daß die Durchgänge der Platte einen Eingang mit einem ersten Radius aufweisen, wobei ein Ausgang mit einem anderen Radius mit axialem Abstand zu dem ersten Radius angeordnet ist.

25. Vorrichtung nach einem der Ansprüche 21 bis 24,
**gekennzeichnet** durch
Mittel zum Erwärmen des Elektrolyten.

26. Vorrichtung nach einem der Ansprüche 21 bis 25,
dadurch **gekennzeichnet,**
daß das Metall in einem Korb in dem Elektrolyten innerhalb der Graphitform enthalten ist.

27. Vorrichtung nach Anspruch 26,
dadurch **gekennzeichnet,**
daß der Korb aus einem leitenden Material gefertigt ist, welches nicht mit Nickel reagiert.

28. Vorrichtung nach Anspruch 26 oder 27,
dadurch **gekennzeichnet,**
daß der Korb aus Titan gefertigt ist.

29. Vorrichtung nach einem der Ansprüche 21 bis 28,
**gekennzeichnet** durch
Mittel zum Ändern des angelegten Stroms.

30. Vorrichtung nach Anspruch 29,
**gekennzeichnet** durch
Mittel zum pulsförmigen Ändern des angelegten Stroms.

## Revendications

1. Procédé de fabrication d'outils de dressage diamantés comportant les étapes consistant à former un moule (10) pour l'outil de dressage, ayant le profil interne (12) voulu, faire adhérer des diamants (14) audit profil, placer le moule dans l'électrolyte, et plaquer par galvanoplastie un métal sur les diamants, caractérisé par le fait que l'opération de placage par galvanoplastie est effectuée pendant qu'un mouvement tourbillonnaire est imparti à l'électrolyte.

2. Procédé selon la revendication 1, caractérisé par le fait que l'électrolyte est pompé à travers le moule.

3. Procédé selon les revendications 1 ou 2, caractérisé par le fait que l'électrolyte est pompé à travers une plaque (24) ayant des passages (26) formant un angle pour l'électrolyte.

4. Procédé selon la revendication 3, caractérisé par le fait que les passages ont une entrée sur un rayon et une sortie sur un autre rayon, espacé axialement du premier rayon.

5. Procédé selon une quelconque des revendications 1 à 4, caractérisé par le fait que l'électrolyte est maintenu à une température supérieure à 35 °C.

6. Procédé selon la revendication 5, caractérisé par le fait que la température de l'électrolyte est maintenue dans la gamme de 39 à 41 °C.

7. Procédé selon une quelconque des revendications 1 à 6, caractérisé par le fait que le métal est du nickel.

8. Procédé selon la revendication 7, caractérisé par le fait que l'électrolyte est du sulfamate de nickel en solution aqueuse.

9. Procédé selon la revendication 8, caractérisé par le fait que la concentration de l'électrolyte est dans la gamme de 550 à 650 g/litre.

10. Procédé selon la revendication 8 ou 9, caractérisé par le fait que l'électrolyte a un pH acide au-dessus de 3,5.

11. Procédé selon une quelconque des revendications 1 à 10, caractérisé par le fait que les diamants adhèrent au profil au moyen d'un adhésif conducteur.

12. Procédé selon la revendication 11, caractérisé par le fait que l'adhésif est un adhésif à base d'argent.

13. Procédé selon la revendication 12, caractérisé par le fait que l'adhésif est un adhésif epoxy à charge d'argent.

14. Procédé selon une quelconque des revendications 7 à 13, caractérisé par le fait que le nickel est sous la forme de grains.

15. Procédé selon une quelconque des revendications 1 à 14, caractérisé par le fait que le placage par galvanoplastie est commencé à un courant bas qui est augmenté graduellement.

16. Procédé selon la revendication 15, caractérisé par le fait que le placage par galvanoplastie est commencé à un courant dans la zone des 2 Ampères.

17. Procédé selon la revendication 15 ou 16, caractérisé par le fait que le courant est augmenté jusqu'à 12 à 14 Ampères.

18. Procédé selon les revendications 15, 16 ou 17, caractérisé par le fait que le courant de départ est maintenu pendant 16 à 24 heures.

19. Procédé selon une quelconque des revendications 1 à 18, caractérisé par le fait que le courant final est maintenu pendant une période de temps jusqu'à 48 heures.

20. Procédé selon une quelconque des revendications 15 à 19, caractérisé par le fait que l'augmentation de courant est pulsée.

21. Appareil de fabrication d'outils de dressage diamantés comportant un bain d'électrolyte pour recevoir un moule de graphite (70) ayant le profil interne voulu recouvert de diamants (71) en tant que cathode, une source de métal (76) en tant qu'anode et des moyens pour faire passer un courant électrique entre l'anode et la cathode grâce à quoi le métal est déposé sur les diamants, caractérisé par le fait qu'il comporte des moyens pour impartir un mouvement tourbillonnaire à l'électrolyte.

22. Appareil selon la revendication 21, caractérisé par le fait que les moyens conçus pour impartir un mouvement tourbilionnaire à l'électrolyte comportent des moyens de pompage.

23. Appareil selon la revendication 22, caractérisé par le fait qu'il comporte une plaque (64) au travers de laquelle l'électrolyte est pompé, la plaque ayant des passages (66) formant un angle à travers elle.

24. Appareil selon la revendication 23, caractérisé par le fait que les passages de la plaque comportent une entrée sur un rayon et une sortie sur un autre rayon, espacé axialement du premier rayon.

25. Appareil selon une quelconque des revendications 21 à 24, caractérisé par le fait qu'il comporte des moyens pour chauffer l'électrolyte.

26. Appareil selon une quelconque des revendications 21 à 25, caractérisé par le fait que le métal est contenu dans un panier dans l'électrolyte à l'intérieur du moule de graphite.

27. Appareil selon la revendication 26, caractérisé par le fait que le panier est fait en un matériau conducteur qui ne réagit pas avec le nickel.

28. Appareil selon la revendication 26 ou 27, caractérisé par le fait que le panier est fait de titane.

29. Appareil selon une quelconque des revendications 21 à 28, caractérisé par le fait qu'il comporte des moyens pour modifier le courant appliqué.

30. Appareil selon la revendication 29, caractérisé par le fait qu'il comporte des moyens pour modifier le courant appliqué de façon pulsée.
